

1

3,676,125

METHOD OF PRODUCING PLANOGRAPHIC  
PRINTING PLATES

Louis Maria de Haes, Edegem, Belgium, assignor to  
Agfa-Gevaert, Mortsel, Belgium  
No Drawing. Filed Apr. 24, 1970, Ser. No. 31,787  
Claims priority, application Great Britain, Apr. 25, 1969,  
21,279/69

Int. Cl. G03f 7/02

U.S. Cl. 96—33

11 Claims

ABSTRACT OF THE DISCLOSURE

A photographic printing plate is prepared from a sheet material carrying an exterior hydrophilic colloid layer having substantially concentrated at its free surface a pattern of finely divided silver particles, by contacting the same with an aqueous alkaline liquid fixer composition containing an oxidizing agent for said silver particles, e.g. cyanoferate(III)-ions, an organic thioxo compound or tautomer thereof for converting the pattern of silver particles into a hydrophobic ink-receptive pattern, a higher fatty acid, e.g., oleic acid, for improving the ink-receptivity of said pattern, and a water-soluble nitrite, such as alkali metal nitrite or an ammonium nitrite, for stabilizing the dispersion of the higher fatty acid in the fixed liquid.

The present invention relates to a method of producing a planographic printing plate by converting a silver image into a hydrophobic ink-receptive pattern.

The preparation of a printing plate according to the present invention comprises treating a sheet material having an outer hydrophilic colloid layer carrying at its surface a pattern of finely divided silver particles, with an aqueous fixer comprising an oxidizing agent for said silver particles, an organic compound that converts the pattern of silver particles in a hydrophobic ink-receptive pattern, a higher fatty acid having from 12 to 22 carbon atoms, and a water-soluble nitrite, the said outer hydrophilic colloid layer having been hardened before, during or after said treatment at least to such an extent that no substantial amounts of colloid are transferred during printing.

The present invention also relates to an aqueous fixer as described above.

The presence of the higher fatty acid in the aqueous fixer results in an improvement of the hydrophobic ink-receptive characteristics of the printing portions. This effect is especially pronounced when the sheet material to be treated with the fixer for the production of the printing plate is a photographic material comprising at its surface a silver pattern, which has been formed according to the silver complex diffusion transfer process from silver complexes diffusing image-wise distributed from an underlying image-wise exposed silver halide emulsion layer. Consequently, the method of the present invention is particularly suited for application in connection with this specific embodiment. However, the higher fatty acid does not remain homogeneously distributed in the fixer and easily tends to unmix during aging. This tendency is fully overcome by the addition of the water-soluble nitrite. Thus, an aqueous fixer having excellent keeping qualities is obtained.

If a water-soluble cyanoferate(III) is used as the oxidizing agent in the fixer, the water-soluble nitrite exerts a further favourable effect in preventing an undesirable yellow, brownish, and even bluish colouring of the fixer during aging. Although such a colour change has no substantial effect on the very fixing properties, it might confuse the operator as to the nature as well as to the quality of the liquid.

2

All water-soluble nitrites, i.e. all organic and inorganic compounds releasing nitrite ions in an aqueous medium are suited for use according to the present invention. Preferably simple water-soluble inorganic nitrites are used, e.g. sodium nitrite, potassium nitrite, or ammonium nitrite. The nitrites are generally applied in an amount comprised between 2 and 20 g. per litre of fixer.

The higher fatty acids to be incorporated into the fixer include saturated as well as unsaturated acids, e.g. lauric acid, myristic acid, palmitic acid, stearic acid, and oleic acid. The unsaturated higher fatty acids and especially oleic acid have proved to be the most suited ones for the purpose of the present invention. These higher fatty acids may be incorporated into the fixer from a solution in a water-miscible organic solvent, e.g. a lower aliphatic alcohol such as propanol, or in the form of a water-soluble salt (soap), e.g. the sodium or potassium salt. A water-soluble salt of the higher fatty acid may also be produced in situ by the presence of suitable alkaline substances such as trisodium phosphate or sodium hydroxide, in the fixer. Thus, the expression higher fatty acids also includes the water-soluble salts thereof. The higher fatty acids are preferably applied in an amount comprised between 5 and 120 g. per litre of fixer.

The oxidizing agent present in the fixer liquid preferably is a water-soluble cyanoferate(III), and the fixer is then preferably buffered at a pH value between 7 and 12.

Suitable organic compounds for converting the pattern of silver particles into a hydrophobic ink-receptive pattern are thioxo compounds, including the tautomeric structures thereof.

For more details on suitable oxidizing agents, specific organic compounds for converting the pattern of silver particles into ink-receptive parts and other usual ingredients of the fixer, and for general data about the production of the silver pattern (preferably according to the silver complex diffusion transfer process) as well as about the preparation and the use of the printing plate reference is made to the U.S. patent specification 3,083,097, and U.S. Pat. 3,582,328 issued June 1, 1970, corresponding to the published Dutch patent application 68/00431, and to the U.S. patent applications Ser. Nos. 887,323, 887,324 and 887,387, now abandoned. The sheet material carrying the silver pattern at its surface (e.g. produced from silver complexes, which have diffused image-wise from an underlying silver halide emulsion layer) preferably comprises a paper support or a hydrophobic synthetic film support including a paper sheet provided with a thin layer of a hydrophobic synthetic polymeric material, e.g. polyethylene.

The essential disclosure of the three applications identified above is reproduced below.

The preparation of printing plates according to the subject matter of such applications comprises treating a sheet material having an outer hydrophilic colloid layer carrying at its surface a pattern of finely divided silver particles, which pattern has been produced in a photographic way by the application of the silver complex diffusion transfer process being carried out with a single photographic material comprising both the silver halide emulsion layer and the substance or substances for promoting the silver deposition from the diffusing complexed silver halide, i.e., the so-called development nuclei, with an aqueous fixer composition containing an oxidizing agent for the silver particles and an organic thioxo compound or tautomer thereof that converts the pattern of silver particles to a hydrophobic ink-receptive pattern, said outer hydrophilic colloid layer being hardened before, during or after the said treatment, and at least to such an extent that no substantial amount of colloid is transferred on printing.

The silver complex diffusion transfer process is especially suited for producing the pattern of silver particles,

since according to this process the silver deposition mainly occurs at the outer surface of the layer provided with the substance or substances for promoting the silver deposition from the diffusing complexed silver halide, i.e., the so-called development nuclei.

According to a first diffusion transfer embodiment, the development nuclei can be supplied to the light-sensitive material by the processing liquid for carrying out the diffusion transfer process. In this case it is sufficient to dispose of a light-sensitive material only, which is provided either or not with a colloid layer on top of the silver halide emulsion layer. The development nuclei will deposit from the processing liquid onto the surface of the light-sensitive material at the development stage and as a result the diffusion transfer silver deposition will also occur at this outer surface of the light-sensitive material. It is the latter diffusion transfer silver image that will be converted into the ink-receptive printing areas of a planographic printing plate and not the silver image resulting from the primary development of the image-wise exposed silver halide.

According to the embodiment wherein the development nuclei are supplied by the processing liquid and preferably according to said embodiment wherein also a colloid layer is provided on top of the silver halide emulsion layer it is also possible to transfer a diffusion transfer silver image containing stratum to a suitable support and to use the resulting material as starting material for the preparation of a planographic printing plate according to the method of the invention. In connection with this method for the preparation of diffusion transfer images, more particularly the embodiment, wherein a colloid layer is provided on top of the silver halide emulsion layer, there can be referred to the United States patent specification 3,335,005.

As a variant of the said first diffusion transfer embodiment the development nuclei for the diffusion transfer image formation, instead of being supplied by the alkaline processing liquid can also be supplied to the light-sensitive material by a special treatment with a separate liquid composition containing such nuclei. This treatment may be the last step in the preparation of the material or a treatment that is carried out after the exposure of the light-sensitive material and before wetting with the alkaline processing liquid for carrying out the diffusion transfer image formation.

According to a further diffusion transfer embodiment the development nuclei may be provided in a colloid layer on top of the silver halide emulsion layer at the preparation stage; in this way a multilayer material is obtained. Such a multilayer material is known among others from the United States patent specifications 2,725,298 and 2,843,485 and from the United Kingdom patent specification 758,627. After the diffusion transfer image formation, the said colloid top layer containing the diffusion transfer silver image is transferred to another sheet thus providing a colloid layer having on its free surface the pattern of finely divided silver particles as required for the preparation of a planographic printing plate according to the method of the invention. This transfer to another sheet may be avoided by substantially or completely concentrating the development nuclei at the free surface of the outer colloid layer of the multilayer material, whereby the diffusion transfer silver deposition substantially takes place at this outer free surface. In this connection there may be referred to the French patent specification 1,569,398.

The development nuclei, instead of being present in the said colloid layer on top of the silver halide emulsion layer, may also be provided between the light-sensitive emulsion layer and the said colloid layer. After the diffusion transfer image formation the said colloid layer is transferred to another sheet material and carries the diffusion transfer silver image on its free surface.

It is also possible to use a multilayer material comprising a light-sensitive silver halide emulsion layer on top of an image-receiving layer containing development nuclei.

Such a multilayer material is described i.a. in United Kingdom patent specification 654,631 and to the United States patent specifications 3,020,155, 3,203,796 and 3,325,284. After the diffusion transfer image formation the light-sensitive emulsion layer may be removed by detaching in an aqueous rinsing bath as a coherent membrane or in flakes, by dissolving or by stripping off either or not by means of an auxiliary sheet, whereupon the colloid image-receiving layer with the silver pattern formed on its surface becomes visible.

In order to obtain at the surface of the outer hydrophilic colloid layer a diffusion transfer silver deposition as high as possible the development nuclei are very often substantially or completely concentrated at the image-receiving side of that layer. This can be very advantageously effected by the application of the development nuclei through an after-treatment of the colloid layer with a liquid composition containing such nuclei. As already mentioned above this liquid composition may be the processing liquid itself for carrying out the diffusion transfer image formation or another aqueous dispersion or solution of said nuclei, which is provided on top of the hydrophilic colloid layer before the diffusion transfer image formation takes place. In order to keep the development nuclei in dispersion a minor amount of a hydrophilic protective colloid is often added to the dispersion. This amount of colloid does not suffice to form a layer and in most cases is hardened at the hardening stage of the hydrophilic colloid layer or by diffusion of hardener from said layer.

The above is a non-limitative list of embodiments for the production of the silver pattern at the surface of an outer hydrophilic colloid layer. The sheet material carrying the silver pattern generally has a rather simple composition and comprises a suitable support such as a usual hydrophobic flexible film support, e.g. a sheet of cellulose triacetate or of polyethylene terephthalate, or a paper sheet provided either directly or indirectly, e.g., by means of a suitable subbing layer, with a hydrophilic colloid outer layer having at its surface a pattern of finely divided silver particles. Often still a silver halide emulsion layer is present between the colloid outer layer and the support and antihalation dyes or pigments are provided.

According to a preferred embodiment, a photographic material is used which in order comprises a support sheet, preferably a paper support or a hydrophobic film support, an antihalation layer, a silver halide emulsion layer and development nuclei on top thereof. If the antihalation layer is gray the correctness of the exposure can be controlled by judging the diffusion transfer image in transmittance before carrying out the fixing step. In order to obtain a diffusion transfer silver deposition that will be sufficiently high, the said photographic material has to be kept for a short while, e.g. for about 10 seconds, in the dark after it has been wetted with the alkaline processing liquid for carrying out the diffusion transfer image formation. The application of the fixer composition may already occur during the period the multilayer material is kept in the dark. However, this application of fixer may also occur thereafter.

For the production of the diffusion transfer silver image a photographic material comprising development nuclei on top of the silver halide emulsion layer may be provided in roller form. After image-wise exposure, e.g. an episcopic exposure in a camera or an exposure through a transparent original in contact with the photographic material, the latter may be guided automatically through a usual processing unit containing the alkaline processing liquid and comprising guiding and driving means as generally known in the art. In order to overcome processing irregularities during the cutting stage of the multilayer material, an empty tray with loose roller, which is lifted by the material during cutting, may be provided between the exposure unit and the processing unit. Another compact processing unit for such a photographic material, in-

cluding the exposure station is described in the French patent specification 1,582,876.

In producing the pattern of silver particles according to the diffusion transfer process at least part of the compounds that are essential or useful for carrying out said process may be provided in the sheet material(s) used. Among these compounds there may be mentioned developing agents, preservatives for these developing agents, complexing agents, stabilizers, alkaline substances, black-toning agents, hardeners, including latent hardeners, and softening agents. By incorporating the greater part or all of these compounds in the sheet material(s) used the aqueous processing liquid can be reduced to an aqueous solution of alkaline substances and even to pure water.

Suitable substances for promoting the silver deposition from the diffusing complexed silver halide are sulphides of heavy metals such as the sulphides of antimony, bismuth, cadmium, cobalt, lead, nickel, silver and zinc. Other suitable salts are the selenides, polysulphides, polysele-nides, mercaptans and thin(II) halides. Heavy metals or their salts and fogged silver halides are suitable too. The complexed salts of lead and zinc sulphides are active alone as well as mixed with thioacetamide, dithiobiuret, and dithiooxamide. Heavy metals, preferably silver, gold, platina, palladium, and mercury may be used in their colloidal form. From these metals the noble metals are the most active ones.

The support of the photographic material comprising the silver halide emulsion layer may be any usual flexible support sheet e.g. a paper sheet or a transparent hydrophobic usual film support, such as a support of cellulose triacetate or of a polyester e.g. polyethylene terephthalate.

The exposure latitude of the photographic material in most cases can be increased considerably and also the image sharpness of the silver pattern and as a consequence thereof, the sharpness of the final result of printing can be improved by applying antihalation dyes or pigments.

These dyes or pigments may be present in the silver halide emulsion layer or in the support, but preferably are incorporated into a layer situated between the silver halide emulsion layer and the support. If a transparent support is used the antihalation dyes or pigments may be applied at the rear side of the material or on top of the emulsion layer dependent on the manner in which the exposure is carried out, viz at the front side or through the support. Preferably a red or black antihalation dye or pigment is used.

Any silver halide emulsion of the negative or direct positive type may be used dependent on the nature of the original to be reproduced. Preferably, however, emulsions of the negative type having a rather high sensitivity of the order as normally required for camera exposure are used. As a matter of fact, although the exposure of the silver halide emulsion layer may be carried out according to any usual technique e.g. in contact, reflectographically, by transmission or episcopically, mostly an episcopic exposure in a camera is carried out, particularly when the development nuclei are provided on top of the silver halide emulsion layer as detailedly described hereinbefore. The silver halide emulsion layer generally comprises an amount of silver halide equivalent to form about 0.5 g. to about 1.5 g. of silver nitrate and preferably amounting only to the equivalent of about 1 g. of silver nitrate. This means a considerable economy of silver halide with respect to the silver halide content of emulsion layers commonly used in the production of diffusion transfer copies. If necessary a suitable subbing layer is provided for strongly adhering the hydrophilic colloid layer(s) to the support sheet.

For the preparation of the hydrophilic colloid outer layer any hardenable hydrophilic colloid may be used. Suitable hydrophilic colloids include gelatin polyvinyl alcohol, casein, carboxymethylcellulose and sodium alginate. Of course, the nature of the hardener used is dependent on the type of hydrophilic colloid to be hardened.

According to a preferred embodiment of the present in-

vention the hydrophilic colloid binder of said outer layer comprises a mixture of a proteinaceous hydrophilic colloid, preferably gelatin, and a hydrophilic colloid that is a latent hardener for said proteinaceous colloid, i.e. that in the alkaline medium wherein the production of the diffusion transfer image takes place hardens said proteinaceous colloid. Suitable hydrophilic colloids of this type are addition products of high molecular weight hydroxyl group-containing compounds with acrolein, described in the United States patent specification 3,382,077 and especially water-soluble hydroxy alkyl esters of alginic acid, particularly propylene glycol esters of alginic acid, described in the United States patent specification 3,378,373. If gelatin is used in the hydrophilic colloid outer layer, it may be submitted to a treatment as described in the United States patent specification 3,089,770 in order to improve the printing characteristics of the planographic printing plate.

Hardening of the hydrophilic colloid binder of the outer layer may occur before, during or after the treatment with the fixer composition and must occur at least to such an extent that no substantial amount of colloid is transferred on printing neither to the rollers for applying water and ink to the printing plate nor to the material to be printed. In other words hardening i.e. insolubilizing in water and strengthening against mechanical damage must occur at least to such an extent that the material obtained can be used as planographic printing plate.

If the said hardening is carried out before the treatment with fixer, it may occur by adding generally known hardening agents for the hydrophilic colloid(s) of the outer layer such as formaldehyde, glyoxal, mucochloric acid and chrome alum to the coating composition of the outer layer, at the surface of which the silver pattern will be produced, and/or to the coating composition of another layer, with which the said outer layer is in water-permeable relationship whereby hardening of the said outer layer takes place by diffusion of hardener from said other layer to said outer layer. When, as already referred to above, a coating composition comprising development nuclei, either or not together with a minor amount of a hydrophilic colloid to keep the development nuclei in dispersion is applied on top of the said outer layer the hardeners can be also be incorporated into said coating composition.

Hardening of the hydrophilic colloid binder of the outer layer may also occur during the production of the silver pattern according to the silver complex diffusion transfer process. Said hardening may occur by incorporating hardeners in at least one of the processing liquids and/or by incorporating latent hardeners, as already referred to above, into the photographic material to be hardened.

Finally, hardening of the outer hydrophilic colloid layer can also occur after the production of the silver pattern namely by treatment with a hardening liquid. This liquid may be an aqueous hardening composition applied before the treatment with the fixer, the fixer composition itself or an aqueous hardening composition applied after the treatment with the fixer.

The presence of certain hydrophilic colloid binders e.g. carboxymethylcellulose, gum arabic, sodium alginate, propyleneglycol ester of alginic acid, hydroxyethyl starch, dextrose, hydroxyethylcellulose, polyvinylpyrrolidone, polystyrene sulphonic acid and polyvinyl alcohol in the outer hydrophilic colloid layer carrying at its surface the pattern of silver particles often improves the hydrophilic, ink-repellent properties of the non-printing areas of the printing plate finally obtained. Also hygroscopic substances likewise called hydrophilic softening agents, e.g. sorbitol, glycerol, trihydroxyethyl ether of glycerol and turkish red oil, and certain wetting agents, i.e. those mentioned hereinafter incorporated in at least one hydrophilic colloid layer of the sheet material carrying the silver image at its surface will improve the hydrophilic properties of the non-printing areas.

The hydrophilic colloid outer layer also may advantageously comprise a considerable amount of pigment particles that will prevent the so-called "scumming" (i.e. ink-acceptance that arises in the non-printing areas of the printing plate after a certain number of copies has been printed). The usual inorganic pigments e.g. barium sulphate, titanium dioxide, china clay and silica applied from a colloidal solution, have proved to be particularly suitable for this purpose. The pigment particles are generally homogeneously applied in such an amount that about 5-20 g. thereof are present per sq. m. of the hydrophilic colloid outer layer. A similar anti-scumming effect may also be obtained by adding at least one member selected of colloidal silica, an inorganic acid e.g. o-phosphoric acid, a hydrophilic softening agent as those mentioned above and a suitable wetting agent to the fountain solution used during the printing process. Suitable wetting agents are i.a.

$\text{H}_3\text{C}-(\text{CH}_2)_{16}-\text{COO}-(\text{CH}_2-\text{CH}_2-\text{O})_5-\text{H}$   
sodium dodecylsulphate  
sodium tetradecylsulphate

$\text{R}-\text{CH}_2-\text{SO}_3\text{Na}$  wherein R represents an alkyl group comprising from 14 to 18 carbon atoms



$\text{R} =$  hexadecyl 90%  
octadecyl 6%  
octadecenyl 4%

A very suitable fountain solution comprises water, glycerol, o-phosphoric acid and colloidal silica.

For the production of the planographic printing plate, the sheet material comprising an outer hydrophilic colloid layer having at its surface a pattern of finely divided silver particles is treated with an aqueous fixed composition as described above.

As disclosed in U.S. Pat. 3,083,097, various oxidizing agents are available for oxidizing the finely divided silver particles in the surface pattern including the water-soluble cyanoferrate(III) compounds mentioned above. Other oxidizing agents include water-soluble  $\text{Cr}^{6+}$  salts, e.g., sodium or potassium dichromate (application S.N. 887-323), water-soluble iron(III) salts, e.g., iron(III) chloride (application Ser. No. 887,324), and water-soluble tin(IV) salts, e.g., tin(IV) chloride, water-soluble cerium(III) salts, e.g., cerium(III) sulfate, and water-soluble persulfates, e.g., potassium persulfate (application Ser. No. 887,387). Where the oxidizing agent is selected from the later groups, the pH of the composition is desirably made acidic by means of a suitable acidic compound e.g., acetic acid or boric acid. A pH of not more than 4.0 is preferable for iron(III) salts and less than 3.5 is preferably for the  $\text{Cr}^{6+}$  salts. The oxidizing agent mostly is incorporated into the fixer composition in a concentration of from 10 to 300 g. per liter. In the case of  $\text{Cr}^{6+}$  salts, the presence of halide ions often has a favorable effect on the action of the fixer composition. So, water-soluble chlorides, bromides or iodides, such as potassium bromide, are often incorporated into the fixer.

The oxidizing agent used in carrying out the present method may be used in combination with at least one other oxidizing agent, e.g., a lead(II) ion-releasing compound,

a water-soluble permanganate, iodic acid, and a compound releasing copper(II) ion as described and claimed in the Belgian patent specification 720,695.

In addition to the oxidizing agent an organic thioxo compound or tautomer thereof that converts the silver image parts in hydrophobic ink-receptive parts is added to the fixer. Examples of such organic compounds that have proved to be especially suitable for this purpose are thioxo compounds, including the tautomeric structures thereof, making the silver image ink-receptive, e.g.

imidazoline-2-thiones and imidazolidine-2-thiones including the N-substituted derivatives such as



imidazolidine-4-on-2-thiones including substituted derivatives such as



tetrahydro pyrimidine-2-thiones including substituted derivatives such as



tetrahydro- and dihydro-oxazine-2-thiones and thiazine-2-thiones including substituted derivatives such as

9

(9)



1,3,4-dihydro thiadiazine-2-thiones including substituted derivatives such as

(10)



thiourea compounds including substituted derivatives preferably N-phenyl thiourea compounds such as

(11)



a compound of another type and that also converts the silver image parts in hydrophobic ink-receptive parts is

(12)



The compounds that convert the silver image parts in hydrophobic ink-receptive parts may be added directly to the fixer, but are often added from an aqueous solution or from a solution in a suitable organic, water-miscible solvent such as ethanol, isopropanol, ethylene glycolmono-methyl ether and dimethylformamide. They must be at least partially soluble in the fixer composition. They are mostly applied in an amount of from 0.5 to 5 g. per litre fixer. It is remarkable that most of the suitable compounds for converting the silver image parts in ink-receptive parts are generally known black-toning agents in the silver complex diffusion transfer process.

An explanation of the reaction mechanism according to which the silver image parts are converted into hydrophobic ink-receptive parts cannot be given with certainty. Indeed, it might be a chemical transformation that takes place or more likely a physical adsorption to the silver image parts. In any event the fact remains that at least a superficial oxidation of the silver pattern is necessary. With certain thioxo compounds it is possible that oxidation products of these compounds are present in the fixer and it is not beyond possibility that precisely these oxidation products are responsible for the hydrophobizing effect obtained in carrying out the method of the invention.

The fixer may comprise some further compounds for improving the hydrophilic ink-repellent properties of the non-printing areas. Suitable such compounds are colloidal silica and hydrophilic colloid binders, hydrophilic softening agents, inorganic acids and wetting agents already mentioned and exemplified above. These compounds mostly are added to the fixer in a concentration ranging from about 5 to about 200 g. per litre.

The fixer may also contain compounds for improving the ink-receptive character of the printing areas such as higher fatty acids, e.g. oleic acid, which often are applied together with a water-soluble nitrite in order to keep them homogeneously distributed in the fixer, and hydrophobic softening agents, e.g. dimethyl phthalate, dibutyl phthalate, the phthalic acid ester with the following formula:



10

triphenyl phosphate, and tricresyl phosphate. The hydrophobic softening agents mostly are added to the fixer in an amount of from about 5 to about 100 g. per litre. It is also possible to apply at least one of these compounds in about the same concentrations after the treatment with the fixer composition.

The fixer composition used in carrying out the method of the present invention is very stable to aerial oxidation and to temperature fluctuations and it may be used for the production of many printing plates without having to frequently adjust the processing time. Many printing plates (about 100 plates of 21 cm. x 29.7 cm. size per litre of fixer) can be produced before the fixer composition is fully exhausted.

At the moment the treatment with the aqueous fixer starts the outer colloid layer showing the silver pattern may be in dry as well as in wet condition. A superficial oxidation of the silver pattern suffices; generally, however, a more penetrating oxidation is advantageous. Generally the treatment with the fixer does not last long, mostly not longer than about 20 seconds and can be accelerated by increasing the concentration of the components in the fixer. The plate may be stored for a long time before being fixed and even thereafter it may be stored for a long time before being used in the printing process. Preferably, however, the fixing step is carried out just before printing.

The fixer as well as the development or activating liquid for the production of the diffusion transfer image can be applied in different ways, e.g. by spraying, by rubbing, with a lick roller, or by dipping the material to be treated in the liquid composition. Also the fixing step of the printing plate may occur automatically by conducting the plate through a device having a narrow channel filled with the fixer composition and at the end thereof between two squeezing rollers. In order to reduce the risk for aerial oxidation of the fixer to a minimum, funnel-shaped in- and outlet openings may be provided at the ends of the narrow channel and an upperlying plastic bag containing the fixer liquid may be used. If the apparatus is not used, the bag is moved downwards and the fixer runs back from the channel into the bag.

The production of a silver image on top of the outer hydrophilic colloid layer (occasionally including the image-wise exposure of the silver halide emulsion layer) and the treatment with the fixer may occur automatically, e.g. in processing stations as described above and occasionally may be carried out both in a compact processing unit comprising both processing stations.

After the application of the fixer the sheet material is ready for use as a printing plate. This means that no further treatment with a lacquer composition for strengthening the printing parts is necessary.

This is an important advantage of the method of the present invention over most of the conventional methods hitherto used for the production of a planographic printing plate that require the application of a lacquer as an essential feature.

Nevertheless, in some cases the hydrophobic character of the ink-receptive parts may still be improved and their mechanical strength may be reinforced by applying a lacquer thereon. Suitable lacquer compositions are solutions of oils, waxes, and resins in organic solvents. Suitable organic solvents are cyclohexanone, acetone, butanol, monomethyl ether of ethylene glycol, monoethyl ether of diethylene glycol, tetrahydrothiophene-1,1-dioxide, diacetone, dioxane, 1,2-dichloroethane, ethyl acetate, trichloroethylene, butyl butyrate, diethanolamine and dimethylformamide. Mixtures of such organic solutions with an aqueous phase or dispersions of such organic solutions in an aqueous phase are suitable too. In that case the aqueous phase may contain thickeners or other usual compounds for improving the hydrophilic character of the non-printing areas of the lithographic printing plate as described above. Suitable lacquers are described in the United Kingdom patent specifications 967,598,

## 11

968,706 and 1,004,342, and in the United States patent specification 3,378,372. Resins that have proved to be especially suitable for improving the ink-receptive character of the printing areas and strengthening them are phenol-formaldehyde resins e.g. the usual phenol-formaldehyde resins, o-cresol formaldehyde resins and p-tert-butylphenol formaldehyde resins, alkyd resins e.g. rosin maleic acid esters, epoxy resins e.g. condensation products of a poly(aryl ethylene oxide) with an acid anhydride, an amine or another suitable compound and epoxidized polyesters.

The resin, wax or oil used mostly is present in a concentration of from about 100 to about 500 g. per litre of liquid lacquer composition. The liquid lacquer composition may be applied after the aqueous composition containing the oxidizing agent has been applied and while the printing plate is still wet. Only when an emulsion lacquer is used the plate need not necessarily be wet at the stage the lacquer is applied. The lacquer may be applied by dipping, spraying, spreading or by means of a material soaked therewith. The lacquer is rubbed out e.g. with a plug of wadding. The hydrophobic solid substances settle on the image areas and improve the hydrophobic ink-receptive character thereof. At the same time the mechanical strength of the printing areas is improved. The adherence of the lacquer to the printing areas may still be improved by heating the plate.

Instead of being applied by means of a separate after-treatment of the printing plate, the liquid lacquer composition may also be mixed with the aqueous fixer composition. The ratio of the organic phase that contains the hydrophobic solid substances to the aqueous phase then mostly is comprised between 1:1 and 1:10.

The printing plate has to be wet at the stage the fatty printing ink is applied. This is generally known in the art and it is usual to apply an aqueous liquid before applying the printing ink. This may occur by means of a wet sponge or by means of the fountain arrangement of the printing machine. This wetting has to be more intensive as the printing plate is drier, e.g., when it has been stored for a long time after its fixation and occasional lacquering.

The following examples illustrate the method and the fixer of the present invention.

## EXAMPLE 1

A thin grey antihalation layer was applied to an extra strong paper support of 135 g. per sq. m. at a ratio of 1 litre per 40 sq. m. with a dispersion of 3 g. of lamp black in 1 litre of a 4% aqueous solution of gelatin.

To this antihalation layer a common high-sensitive silver chlorobromide gelatin emulsion layer comprising hydroquinone and 1-phenyl-3-pyrazolidinone was applied in such a way that per sq. m. were present: an amount of silver halide equivalent to 1 g. of silver nitrate, 1 g. of hydroquinone, and 0.5 g. of 1-phenyl-3-pyrazolidinone.

The following coating composition was applied to the dry silver halide gelatin emulsion layer in a ratio of 100 g. per sq. m.:

Water—926 ml.

Gelatin—10 g.

12.5% aqueous saponin—8 ml.

20% aqueous formaldehyde—56 ml.

Then the following liquid was applied at a rate of 22 g. per sq. m.:

Water—890 ml.

12.5% aqueous saponin—10 ml.

Aqueous dispersion of colloidal nickel sulphide nuclei comprising per 100 ml. 0.2 g. of nickel sulphide and 10 g. of gelatin—100 ml.

The light-sensitive multilayer material thus obtained was image-wise exposed to an original.

## 12

After the image-wise exposure the multilayer material was guided through a processing unit containing the following alkaline liquid:

5 Water—1000 ml.  
Sodium phosphate-12-water—75 g.  
Anhydrous sodium sulphite—40 g.  
Potassium bromide—0.5 g.  
Anhydrous sodium thiosulphate—10 g.

10 Subsequently, the multilayer material was kept for approximately 10 seconds in the dark to make possible an intense silver deposition by diffusion transfer. A sharp bronzed legible diffusion transfer image became visible on a gray background.

15 The plate was then rubbed for approximately 20 seconds with the following fixer:

Water—50 ml.  
Trisodium phosphate-12-water—4.0 g.  
Potassium cyanoferrate(III)—9.8 g.  
20 Ethylene glycol monoacetate—5 ml.  
n-Propanol—20 ml.  
Oleic acid—3.0 ml.  
Sodium nitrite—0.5 g.  
10% solution of 1-allyl-imidazolidine-2-thione in ethylene glycol monomethyl ether—5.2 ml.  
25 Distilled water up to—100 ml.

The pH of this buffered fixer composition was 7.6. A high-quality planographic printing plate having positive image values in respect of the original was obtained.

30 The fixer described above has excellent keeping qualities. The colour of the fixer does not change during aging and the oleic acid remains homogeneously distributed throughout the fixer. A similar fixer containing, however, no sodium nitrite becomes brownish and bluish after about one week, and the oleic acid unmixes from the aqueous phase. Said unmixing is of course highly unwanted since it impairs the fixing properties.

## EXAMPLE 2

35 Example 1 was repeated with the difference, however, that trisodium phosphate-12-water was omitted from the fixer and oleic acid was replaced by 3 g. of the sodium salt of oleic acid. The fixer thus obtained has a pH-value of 8.8 and shows good keeping properties which are similar to those of the fixer described in Example 1.

40 By proceeding in this way a high-quality printing plate was obtained.

I claim:

50 1. Aqueous fixer liquid composition for use in the production of a planographic printing plate from a sheet support having an outer hydrophilic colloid layer carrying substantially concentrated at its free surface a pattern of finely divided silver particles, said fixer comprising an oxidizing agent for said silver particles, an organic thioxo compound or tautomer thereof adapted to convert the pattern of silver particles into a hydrophobic ink-receptive pattern, a higher fatty acid having about 12-22 carbons in the fatty chain dispersed in said aqueous liquid in an amount sufficient to improve the hydrophobic characteristics of said ink-receptive pattern, and a water-soluble nitrite in sufficient amount to significantly improve the stability of the fatty acid dispersion.

55 2. Aqueous fixer composition according to claim 1, wherein the fatty acid is an unsaturated higher fatty acid.

3. Aqueous fixer composition according to claim 1, wherein the higher fatty acid is present in an amount of between 5 and 120 g. per litre of fixer composition.

60 4. Aqueous fixer composition according to claim 1, wherein the water-soluble nitrite is present in an amount of between 2 and 20 g. per litre of fixer composition.

65 5. Aqueous fixer composition according to claim 1, wherein the oxidizing agent is a water-soluble cyanoferrate(III) and the fixer composition is buffered at a pH value between 7 and 12.

6. In the method of producing planographic printing plates which comprises contacting a sheet support having an exterior hydrophilic colloid layer carrying substantially concentrated at its free surface a pattern of finely divided silver particles, with an aqueous alkaline fixer composition containing an oxidizing agent for said silver particles, and an organic thioxo compounds or a tautomer thereof adapted to convert the pattern of the oxidized silver particles into a hydrophobic ink-receptive pattern, the improvement of incorporating in said fixer composition an amount of dispersed higher fatty acid having about 12-22 carbons in the fatty chain thereof sufficient to improve the hydrophobic characteristics of the ink-receptive pattern together with a sufficient amount of a water-soluble nitrite to significantly improve the stability of the dispersion of said fatty acid.

7. A method according to claim 6, wherein the higher fatty acid is present in an amount of between about 5-120 g., and the water-soluble nitrite in an amount of about 2-20 g. per liter in the fixer composition are used and said solution is buffered at a pH value of about 7-12.

8. A method according to claim 6, wherein the pattern of silver particles is produced according to the silver complex diffusion transfer process.

9. A method according to claim 8, wherein the silver pattern has been formed from image-wise distributed silver complexes diffusing from an underlying image-wise exposed silver halide emulsion layer.

5 10. A method according to claim 6, wherein the sheet support is a paper support, hydrophobic synthetic film support, or a paper sheet provided with a thin layer of a hydrophobic synthetic polymeric material.

10 11. A method according to claim 6, wherein the higher fatty acid is an unsaturated higher fatty acid selected from the group consisting of lauric acid, myristic acid, palmitic acid.

#### References Cited

##### UNITED STATES PATENTS

3,083,097 3/1963 Lassig et al. ----- 96-29 L  
3,260,198 7/1966 Wagemans et al. ----- 96-29 L

DAVID KLEIN, Primary Examiner

U.S. CL. X.R.

96-29 L; 101-466